

Patented May 29, 1923.

1,457,102

# UNITED STATES PATENT OFFICE.

FRANCIS BRADLEY AND HARRY L. FREVERT, OF PHILADELPHIA, PENNSYLVANIA.

## ARMOR PLATE AND PROCESS OF MAKING SAME.

No Drawing.

Application filed June 27, 1922. Serial No. 571,302.

To all whom it may concern:

Be it known that we, FRANCIS BRADLEY and HARRY L. FREVERT, citizens of the United States, residing at Philadelphia, county of 5 Philadelphia, and State of Pennsylvania, have invented a new and useful Improvement in Armor Plates and Processes of Making Same, of which the following is a full, clear, and exact description, reference 10 being had to the accompanying drawings, which form a part of this specification.

In an application filed by us June 27, 1922, Serial No. 571,301, we set forth the discovery that if armor plate which is already 15 treated, by known methods, to produce a plate having a hardened front with a carburized face, and a tough back, is drawn at a temperature above 500° F. and below 1100° F., so as to remove from the hard 20 front practically all the brittleness and a large portion of the hardness, while maintaining the stiffness required to offer extraordinary resistance to displacement, it will offer greater resistance to penetration, 25 with projectiles of the present improved type, than is offered by a plate of the ordinary type, wherein the hard front of the plate is unable to break the point of the projectile and is itself cracked and spalled off 30 with less expenditure of power than would be required were the metal to remain in position and offer great resistance to displacement.

The object of the present invention is to 35 improve the process set forth in the above application for patent by still further increasing the resistance of the plate to perforation and at the same time prevent cracking under the shock of impact.

A plate of the type to which our invention 40 is applicable may be produced, for example, by the following process, well known to those skilled in the art: An ingot of any suitable composition is cast, and after reheating is 45 forged or rolled into a plate of a thickness about 20% in excess of the thickness desired for the finished plate. The plate, thus formed, may be reheated and annealed, or reheated to below the critical temperature 50 and cooled either quickly or slowly. The side of the plate intended for the face is then cleaned of all scale and a brick container built around its edges. The container is filled with a suitable carburizing compound, and a similar plate is laid face down 55 upon it, the pair of plates being then heated

to a temperature and for a time suitable for penetration of carbon into the face of the plate, to the desired depth and extent, or the plate may be carburized by a gas. 60

After the carburization of the plate, by the absorption thereby of the desired carbon, the plate is carefully cooled, and freed of scale, the face protected by a carbonaceous covering, reheated to a very low forging 65 temperature and forged to final thickness. The plate is then reheated to a temperature considerably above its critical temperature, quenched, again reheated, but to a less degree than before and again quenched; the 70 plate is then again reheated to a point below its critical temperature, bent and cooled slowly; again reheated to a point well below its critical temperature and quenched. The face of the plate is then heated rapidly 75 to well above its critical temperature, while the back is kept below that temperature and the plate quenched throughout. In this heating operation, the temperature of the plate is raised to above the critical temperature to a depth substantially exceeding the 80 relatively thin carburized face zone and it is this part of the plate, which includes the carburized face and a zone to the rear thereof, which I call the "front." 85

In the above described and other well known processes of face hardening armor plate it is present practice to harden to a depth, in the case (say) of a 13½ inch plate, of substantially less than five inches to not 90 over about six inches or from thirty-five to less than forty-five per cent of the thickness of the plate. Increase of the hardened zone, in the case of plates of the present type, would not only not give greater re- 95

sistance to penetration, but would be detrimental, as it would provide a disproportionately thin tough back. In manufacturing our improved armor plate, however, we find that if the plate (say 13½ inches in thickness) is hardened to a depth varying from substantially over six inches to nearly nine inches, or from at least forty-five per cent to about sixty-five per cent of the thickness 100 of the plate, and is then drawn at a temperature of from 500 to 1100 degrees F. (preferably 650 degrees F.), the resistance of the plate to perforation will be still further increased, while, by reason of the removal of the brittleness and a large portion of the 110 hardness from the initially hardened plate, the tough or ductile zone at the back is suf-

ficiently thick to prevent cracking of the plate under shock of impact.

The hardening of the plate to the depth specified is effected by the same methods, 5 well known to those skilled in the art, generally used for hardening the plate to a substantially less depth.

In producing the initially hardened plate, we first carburize the face to a depth of 10 (preferably) from seven to ten per cent of the thickness of the plate.

This application is a continuation in part of application Serial No. 505,888, filed October 6, 1921.

Having now fully described our invention, what we claim and desire to protect by Letters Patent is:

1. The process of so treating armor plate as to render it resistant to perforation, 20 which comprises treating the plate to pro-

duce a tough back and a carburized face hardened front to a depth of from forty-five to sixty-five per cent of the thickness of the plate, and then drawing the plate at a temperature not below 500 degrees F. nor above 1100 degrees F. 25

2. As a new article of manufacture, an armor plate provided with a tough back and a stiff carburized hardened front from which the normal brittleness has been substantially removed and whose normal hardness has been substantially diminished, the depth of the de-brittled, stiff zone of reduced hardness being from forty-five to sixty-five per cent of the thickness of the plate. 30

In testimony of which invention, we have hereunto set our hands, at Philada., Penna., on this 21st day of June, 1922.

FRANCIS BRADLEY.  
HARRY L. FREVERT.